

April 29, 1930.

A. GUNTHARD

1,756,739

APPARATUS FOR APPLYING A SOFT METAL SURFACING TO HARD METAL PLATES

Filed Sept. 7, 1928



WITNESSES

*James Maylor*  
*Hugh H. Ott*

INVENTOR  
*August Gunthard*  
BY  
*Murphy*

ATTORNEY

## UNITED STATES PATENT OFFICE

AUGUST GUNTHARD, OF ARCOLA, NEW JERSEY, ASSIGNOR TO THE CHEMICAL EQUIPMENT MANUFACTURING COMPANY, OF PATERSON, NEW JERSEY, A CORPORATION OF NEW JERSEY

## APPARATUS FOR APPLYING A SOFT-METAL SURFACING TO HARD-METAL PLATES

Application filed September 7, 1928. Serial No. 304,602.

This invention relates to the art of coating hard metals with soft metal, and pertains more particularly to a method of and an apparatus for applying the soft metal 5 facing to hard metal plates, sheets or strips.

At the present time containers or receptacles used in the chemical industry which are constructed of steel and which are provided with a soft metal coating or lining such 10 as lead, are produced almost entirely by hand methods, in which the coating or lining in a soft or fluid state is placed upon or within a receptacle and subsequently smoothed off by a finishing operation.

15 The present invention comprehends a method of applying the coating onto the sheets, strips or plates from which the receptacle is to be subsequently constructed, by flowing said substance while in a fluid molten 20 state onto the plate while the same is being fed successively over a heating medium and subsequently over a cooling medium and providing means for automatically smoothing off the coating substance to a uniform 25 thickness or depth prior to the same reaching the point of cooling.

The invention further aims to provide a simple, effectual and inexpensive apparatus for accomplishing the method set forth.

30 With the above recited and other objects in view, reference is had to the following description and accompanying drawing, in which there is exhibited one example or embodiment of the invention, while the claims 35 define the actual scope of the same.

In the drawing—

The figure is a diagrammatic longitudinal sectional view of the apparatus illustrating the manner in which the plates, sheets or strips are coated.

40 Referring to the drawing by characters of reference, the apparatus employed includes a pair of superposed rollers 10 and 11 and a longitudinally spaced pair of superposed rollers 12 and 13. Adjacent the lower roller 11, a battery of burners or heating pipes 14 are provided for directing upwardly flame jets to heat from the under side a blade, sheet 45 or strip A of the material which is to be coated with the coating B. Adjacent the lower

5 roller 13, a battery of pipes 15 having outlets 16 for directing against the under side of the plate, sheet or strip A cooling blasts, is provided. The apparatus further includes between the heating and cooling means a 55 baffle element 17. At the point where the sheet, strip or plate A is subjected to the action of the heating means 14, the coating substance C is caused to gravitationally flow onto the upper surface of the plate from a suitable 60 source of supply 18, it being understood that the coating is in a molten fluid state. The rollers 10, 11, 12 and 13 are caused to rotate in the directions indicated by the arrows in any desired manner for effecting the feeding 65 of the plate horizontally through the apparatus. Immediately prior to reaching the point where the plate is cooled by the cooling means 15, a doctor plate or scraper 19 is disposed for smoothing the same off to a uniform thickness or depth. After passing this point, the coating under the action of the cooling means 15 hardens or solidifies and adheres to the surface of the plate, strip or sheet 70 A. The rollers 12 and 13 thus cooperate with 75 the coated strip, sheet or plate and feed the same therebeyond. If desired, the upper surface of the coating B may be further subjected to a smoothing action by a rotary cutter or cutters 20 provided for the purpose. 80 If desired, the source of supply 18 or the discharge outlet thereof may be caused to move laterally or transversely with respect to the path of movement of the plate, sheet or strip A, and likewise the cutting element 20 for 85 smoothing the same may be caused to move laterally to the path of movement of the plate.

The method employed consists essentially in applying a soft metal coating to hard metal 90 plates, sheets or strips by feeding the plates horizontally over a heating medium and a cooling medium successively, flowing the coating substance while in a heated fluid state onto the plate at the point of heating and 95 finally smoothing the same off to a uniform thickness or depth prior to reaching the point of cooling and solidifying.

By use of the apparatus heretofore specified and by following the method outlined, it is 100

obvious that the sheets, strips or plates may be coated by a continuous operation to effect a material saving over the hand operation and to obtain a more uniform coating than can be accomplished by the hand methods. It is also apparent that the plates, sheets or strips when coated may be bent or otherwise formed into containers or receptacles for use in the chemical industries.

10 What is claimed is:

1. An apparatus for applying a soft metal coating or surfacing to hard metal plates, sheets, strips or the like comprising means for feeding the same horizontally in a given direction, means below the plate for progressively heating and cooling the same in the direction of its movement, means for flowing onto the plate at its initial point of heating the coating substance while in a heated fluid state and means for smoothing off the upper level of the coating while heated to a uniform thickness or depth.
2. An apparatus of the character set forth comprising a plurality of pairs of driven superposed feeding rollers adapted to coat with a plate, sheet or strip to be coated for feeding the same in a given direction, subterposed means for heating the plate initially, superposed means for flowing a coating substance while in a heated fluid state onto the plate at the point of heating, subterposed means for subsequently cooling the plate and superposed means for smoothing off the coating while heated to a uniform thickness.
3. An apparatus of the character set forth comprising a plurality of pairs of driven superposed feeding rollers adapted to coat with a plate, sheet or strip to be coated for feeding the same in a given direction, subterposed means for heating the plate initially, superposed means for flowing a coating substance while in a heated fluid state onto the plate at the point of heating, subterposed means for subsequently cooling the plate, superposed means for smoothing off the coating while heated to a uniform thickness or depth, baffle means interposed between the heating and cooling means for insulating the same from each other.

50 AUGUST GUNTHARD.